

## UNITED STATES PATENT OFFICE.

WILLIAM E. RUDER, OF SCHENECTADY, NEW YORK, ASSIGNOR TO GENERAL ELECTRIC COMPANY, A CORPORATION OF NEW YORK.

## PROCESS OF TREATING MAGNETIC MATERIAL.

No Drawing.

Application filed January 23, 1924. Serial No. 688,090.

The present invention relates to magnetic steel such as used, for example, in the manufacture of transformer cores, dynamo-electric machinery and the like, and my invention comprises a method of treating steel sheets to improve their magnetic properties, and an improved product resulting from this method.

I have discovered that when sheets of magnetic steel are treated so as to remove a surface layer upon the sheets, as by pickling in acid, in conjunction with an annealing treatment under deoxidizing or purifying conditions, as in a vacuum, or in a reducing but not carburizing gas, regardless of the order in which these steps are carried out, the magnetic permeability is increased and the energy loss during operation is decreased. By the expression "not carburizing" I mean a gas which will not give up carbon to the sheet steel material which is subjected to the action of the gas.

Alloy steel, of which steel containing about three to five per cent of silicon is a conspicuous example, is prepared for use by rolling ingots of steel into sheet form by methods which are well known. Apparently a surface skin of the metal is modified by the rolling process so as to be less susceptible to a subsequent annealing treatment whereby the magnetic properties of the sheets are improved. Whether it is a fact or not that such a surface layer exists (other than the usual surface scale) is difficult to demonstrate by tests other than the undoubted improvement of magnetic properties of the sheets due to its removal in accordance with my invention.

Prior to my invention pickling of silicon steel has been practised with some beneficial effect which was due to the removal of a useless surface scale of oxide. Its removal resulted in a better space factor in the finished apparatus, but no substantial improvement of the steel itself resulted. My experiments indicate that when the pickling was followed by an anneal in contact with gases such as carbon monoxide, this gas undid whatever benefit had been obtained by pickling. Even when closed annealing pots were used, carbon monoxide was in contact with the steel. It now appears that the pickling treatment left the steel in a condition peculiarly susceptible to gases which are present

in ordinary annealing furnaces, and that these gases had a deleterious effect.

When carrying out the process constituting my invention the annealing treatment which either precedes pickling or follows pickling, is carried out under conditions which will not permit of the absorption of deleterious gases.

The surface removal treatment which constitutes the first step of my invention preferably is carried out after the completion of the rolling operation by pickling the alloy steel sheets in accordance with the well understood methods used for removing the scale of ordinary iron and steel parts prior to the usual finishing steps such as galvanizing, japanning, or enameling. For example, the sheets may be immersed in an aqueous solution containing about ten to twenty per cent sulphuric acid. Solutions of hydrochloric or other acids also may be used. The pickling is continued until the scale on the sheets is completely removed. This scale is formed during rolling and usually is thin but is closely adherent. During the removal of the scale from all parts of the surface, a thin layer of the underlying metal also is removed. Usually about fifteen minutes is a sufficient length of time for pickling, but some conditions may require a longer time. The sheets then are washed, dried and annealed in a vacuum or in hydrogen gas at about 800 to 850 degrees centigrade for about one hour. The annealing process may be carried out in a furnace such as described in my prior Patent No. 1,110,010 of September 8, 1914. As therein described, the material is rendered non-oxygenous and of improved magnetic characteristics.

By the described treatment the permeability of the sheets as compared with material which has not been pickled, is increased about ten per cent at working density of magnetic flux and the hysteresis watt losses are decreased about ten to fifteen per cent, depending on the condition of the steel.

In some cases the steel may be annealed prior to pickling, preferably after all the mechanical work such as rolling and punching has been done on the sheets. Preferably, the process described in my prior Patent No. 1,110,010 is employed for the anneal, although the annealing temperature need not necessarily be any higher than 800 to 850 de-

grees centigrade. After anneal the sheets are pickled as above described. In this case, the improvements in permeability and watt loss are even greater than when the anneal follows pickling. Permeability at working density is increased about fifteen per cent and the watt loss is decreased about twenty per cent as compared with the same steel treated by methods previously used involving pickling followed by an anneal which did not remove gases of a harmful nature, which are present in the steel or prevent access of deleterious gases to the steel sheets during anneal.

15. What I claim as new and desire to secure by Letters Patent of the United States, is:

1. The method of improving the magnetic properties of silicon steel sheets which consists in removing a surface layer from said sheets in conjunction with an anneal under conditions favorable to the production of a substantially non-oxygenous condition therein.

2. The method of treating silicon steel sheets which consists in pickling said sheets in an acid bath to remove a surface skin, and annealing said sheets under conditions favorable to the removal of deleterious gases.

3. The method of treating silicon steel

sheets which consists in removing a surface film from said sheets and annealing said sheets under reducing but not carburizing conditions.

4. The method of treating rolled silicon steel sheets which consists in pickling said sheets in an acid bath to remove a surface film and annealing said sheets under reducing but not carburizing conditions.

5. The method of treating rolled silicon steel sheets which consists in pickling said sheets in dilute acid until a surface film has been removed and annealing said sheets in the presence of hydrogen at about 800 to 850 degrees centigrade.

6. The method of improving the magnetic properties of alloy steel sheets which comprises pickling the sheets to remove a surface film and annealing the sheets under reducing but not carburizing conditions.

7. The method of improving the magnetic properties of alloy steel sheets which comprises removing a surface layer from said sheets and annealing the sheets under conditions favorable to the removal of deleterious gases.

In witness whereof, I have hereunto set my hand this 22nd day of January, 1924.

WILLIAM E. RUDER.